

Jan. 2, 1934.

F. A. FAHRENWALD

1,941,672

BRAKE SHOE AND METHOD OF MAKING THE SAME

Filed Jan. 6, 1930



Frank A. Fahrenwald

Executor

by. M. B. E. L.  
Attorney

## UNITED STATES PATENT OFFICE

1,941,672

BRAKE SHOE AND METHOD OF MAKING  
THE SAME

Frank A. Fahrenwald, Chicago, Ill., assignor to  
The American Brake Shoe and Foundry Com-  
pany, New York, N. Y., a corporation of Dela-  
ware

Application January 6, 1930. Serial No. 418,786

14 Claims. (Cl. 148—21.7)

This invention relates to metal brake shoes and the method of making same.

Considering as an example, but without limiting myself thereto, the requirements and conditions encountered in railway practice, it is necessary that a brakeshoe shall develop a certain degree of friction in contact with steel or chilled-iron wheels without unduly wearing or injuring the tread or surface to which it is applied or itself becoming disintegrated in the process. It is also necessary to consider and provide for the extreme local heating produced by the friction of the brakeshoe which very frequently causes the brakeshoes to become red hot, and on some occasions actually leads to melting at localized portions of the working surface. This local heating produces various peculiar and unexpected effects which I will shortly describe.

Plenty of hard and tough alloys are known but the same are unsuitable for brakeshoe use for various reasons, chief among which are that they do not afford proper friction, or that they unduly abrade and damage the surfaces to which they are applied; added to which they are relatively too expensive. The essential requisites for a metal brakeshoe are that it should exhibit a required degree of hardness, coupled with sufficient toughness to withstand the strains and shocks incident to use, and also possess such a texture as to prevent what is known as flaking or undue flowing of the metal surface under the combined heating and abrading effect of the companion part. It is believed that the presence of graphite in the material is of importance in this connection. Ordinary gray cast-iron exhibits all of these requirements to a very satisfactory degree, excepting the qualities of toughness, strength, and wear resistance. The cheapest kind of gray cast-iron, in point of coefficient of friction and cost per pound, serves the purpose better than almost any other metallic substance, but it has the disadvantage of rapid wear and the liability to fracture.

Owing to the effect of local heating and cooling, and to the inevitable formation of surface cracks adjacent the heated surface due to unequal heating, to the variable heating of the brakeshoe which causes the same to change in shape under different conditions of service application, and to looseness of the brake gear which causes the wear of the shoes to become localized at different points, the brakeshoe often breaks long before it is worn out; which is to say that heretofore the life of a brakeshoe has been limited by its brittleness and lack of tensile strength, rather

than by its wear resistance, and to hold the parts of a broken shoe together and prevent them from falling away it has long been customary to cast steel reinforcements in the shoe.

It is well known that cast-iron exhibits no ductility whatever and that no heat treatment thereof will render it ductile, yet a very small degree of ductility imparted thereto would overcome almost all objections to cast-iron brakeshoes.

Accordingly it is the object of my invention to produce a brakeshoe which shall retain substantially the cheapness and composition and friction-coefficient of cast-iron combined with the toughness and tensile strength and ductility of steel; and to do all the foregoing without changing in any way the standard shape, size, and method of attachment of the brakeshoes heretofore adopted and standardized; it is another object of my invention to dispense with the necessity for using inserts or reinforcements; other objects are the provision of a method of making a tough cast-iron brakeshoe without increasing its cost substantially; while further objects and advantages will become apparent as the description proceeds.

It is well known that the treads of car-wheels are often made of what is known as "chilled white-iron", namely a cast-iron containing such proportions of carbon and silicon as when cast against a cold metal surface shall produce what is known as "white-iron", which exhibits phenomenal hardness and abrasion resistance coupled, however, with a very high degree of brittleness and a deficient amount of tensile strength. Attempts to employ this material for brakeshoe purposes have proven unsuccessful because of its unduly small frictional effect, and because of its brittleness and lack of tensile strength which unfit it for the violent shocks and severe operation conditions to which brakeshoes are subjected.

It has also been found that when such material is used for brakeshoes, the local heating at the working surface sets up such strains as to fracture the entire shoe, due to its fragility. Sand-cast white-iron, namely iron which casts white in sand molds owing to a reduction in the amount of carbon and/or silicon, exhibits the same defects when applied to brakeshoe use. Attempts have been made to employ steel, and what is known as "malleable cast-iron", but these attempts have proven unsuccessful chiefly because of the tendency of these substances, under the frictional effect of the car-wheel, to flow and to disintegrate in the form of flakes. Their friction effect is unreliable owing to the local soften-

ing and flowing away of the brakeshoe material under severe conditions; and furthermore experience shows that they wear the car wheel faster than gray-iron.

- 5 There is a type of iron, intermediate between the gray-iron and the white-iron, which I herein call "mottled-iron" since it exhibits a kind of mottled appearance due to the coexistence in the same article of regions of white-iron and regions 80  
10 of gray-iron. My tests have shown that brakeshoes made of this "mottled-iron" retain substantially all the high friction of the gray-iron, together with one advantage of white-iron, namely, increased wear-resistance although, when 85  
15 made by direct casting methods, they still retain the brittleness and fragile nature of the ordinary cast-iron. The one advantage of such mottled-iron is longer wear, but it has been impossible heretofore to produce brakeshoes of this 90  
20 "mottled-iron" by usual casting methods owing to the accurate control of composition and temperature necessary to be exercised and, furthermore, the mottled-iron as produced by casting methods has little, if any, superiority in strength 95  
25 over gray or white-iron. However, I have discovered a mode of producing brakeshoes of cast-iron which shall combine the friction qualities of gray-iron, the wear-resisting qualities of mottled-iron, and the toughness and ductility 100  
30 of steel, and this at a cost as low or even lower than is required in the production of ordinary gray-iron brakeshoes.

To effect this I first cast the brakeshoes at least in part of chilled-white iron, and then by 35 maintaining the castings at the proper temperature for the necessary period of time I cause such a controlled decomposition of the primary cementite thereof with liberation of secondary graphite as shall afford the graphite material desirable for the service of the brakeshoes as above described while retaining such a proportion of the cementite as to afford the desired 40 increase in resistance to wear; and I also anneal or temper the steel matrix in such wise as to decrease its brittleness and render it tough and strong. The results of this treatment and the 45 temperatures and times required to perform the same vary with the composition of the iron and the method of casting employed, although in one 50 respect the result is largely independent of either the composition or the foundry practice, namely: the usual gray cast-iron has very little tensile strength and practically no elongation, due to the shape and arrangement of the graphite 55 particles, while, due to the rounded or nodular shape of the graphite masses resulting from my process the strength is much increased.

The customary brakeshoe composition at the present day is approximately:

|              |               |
|--------------|---------------|
| 60 Carbon    | 2.80 to 3.10% |
| Silicon      | .60 to 1.20%  |
| Phosphorus   | Up to .70%    |
| Sulphur      | Up to .25%    |
| 65 Manganese | Less than 1%  |
| Balance iron | %             |

70 This is a composition which in small sections will produce white-iron, even when cast in sand-molds; a brakeshoe (for example the standard freight-car size of 13 $\frac{3}{4}$  by 3 $\frac{3}{8}$  by 1 $\frac{1}{2}$  inches, weighing twenty pounds) cast therefrom in sand will lie on the borderline between gray-iron and white-iron, at times giving rise to a localized "mottled" condition heretofore mentioned.

According to my improvements I cast these brakeshoes in white-iron, for example, by employing essentially the same composition of melt, the same raw materials, the same cupola practice as at present, but using molds which are made of metal, at least in part, such for example as a mechanical casting machine. After casting I subject the shoes to a temperature of about 1700° Fahrenheit for a period of time of from one to six hours, and afterwards cool them slowly through the critical range, after which the remaining cooling can be at any convenient speed. The result of this first heat treatment at the time and temperature mentioned is to break down the combined carbon partly into graphite, retaining a substantial proportion of the hardness and wear resistance of the white-iron while overcoming sufficient of the brittleness to avoid the objections heretofore made to white-iron, and producing a degree of friction coefficient substantially the same as that of mottled-iron. 90  
95

The breaking strength of a gray-iron or a mottled-iron brakeshoe of the above dimensions as heretofore made has seldom been as high as 100 20,000 pounds even when new and is more frequently around 17,000 pounds. A similar brakeshoe made according to my process and tested in the same manner ordinarily shows a breaking strength of from 23,000 to 26,000 pounds with an 105 increase of useful life of 100 percent or more. It may be stated, in another way, that these shoes can be so made as to exhibit the wear-resistance of white-iron coupled with the friction coefficient of gray-iron and a type of toughness heretofore not possessed by either type of iron, so that their useful life is not, as heretofore, terminated by premature fracture. 110

I have described heat treatment of from one hour to six hours at 1700° Fahrenheit, but these 115 are approximately the extreme time limits at this temperature with the composition described. It is important in my estimation to stop the heat treatment before all of the white-iron condition has been broken down because if carried too far 120 it will produce the customary inferior qualities of malleable-iron brakeshoes, while if not carried far enough it will exhibit the unsatisfactory conditions of white-iron brakeshoes. Preferably, with the composition described, I employ a heat 125 treatment of from three to four hours at 1700° Fahrenheit. The same amount of reaction can be produced by subjecting the brakeshoes to lower temperatures for a longer time or to higher temperatures for a shorter time. However, the 130 time necessary for treatment varies very greatly with the temperature. Maintaining a brakeshoe of this composition at a temperature of 1800° Fahrenheit one hour is excessive for the best results with iron of this specification, and 135 fifteen to twenty minutes seems to be about right, depending of course upon the rapidity of heating and cooling, but such severe conditions are difficult to control or arrest at the desired point. Subjection of this composition to temperature 140 of 1600° Fahrenheit for eight hours yields a material of high wear resistance but somewhat deficient in friction coefficient, and I therefore consider this temperature less desirable because of the long processing required, although it can 145 be used with the right composition of melt, and is sometimes desirable in case it is possible to remove the shoes from the molds at a sufficiently high temperature so that they can be heat-treated by their own retained heat, being placed 150

in a thermally insulated receptacle in large numbers to soak in their mutual heat.

It will be understood that the time and temperature required will vary with the composition of metal employed. Thus if the amount of silicon be increased (or fortified by other ingredients having the same general effect as silicon e. g. nickel, copper, or aluminum) the temperature and/or time of treatment can be decreased somewhat; while if the amount of silicon be decreased relative to the carbon, or if ingredients be introduced having an opposite effect to that of silicon (e. g. chromium, vanadium, or manganese) it may be necessary to increase the time or temperature or both.

In the practical performance of my improved process I preferably employ a casting machine because of the economy of labor and the uniformity of speed and temperature control obtainable thereby. For purposes of speed and heat economy the casting machine is preferably located in such proximity to the heat-treating furnace as to cause the castings to be delivered into that furnace substantially at the desired temperature. Preferably they are discharged directly onto a traveling conveyor whose speed of movement is so adjusted as to remove them from the heated chamber after the lapse of the desired heating interval and carry them through subsequent chambers decreasing in temperature at a predetermined rate, whereby they are cooled through the critical temperature at the desired speed for the structure and toughness desired. It should be noted that the mere subjection of the castings to the first or high temperature heat treatment, while sufficient for the development of some qualities, exhibits its full advantages only when followed by a controlled cooling through and adjacent to the critical range. The treatment at the high temperature fixes the proportions of cementite and graphite; the cooling from this higher temperature down through the critical range determines the relation of hardness to toughness in the matrix metal.

The secondary graphite liberated during the high temperature treatment appears in the form of compact nodules of irregular outline embraced by a steel-like matrix; the extent of the graphitizing depends on the temperature and time and should not be carried to completion but only until the desired friction-coefficient is attained and before the matrix metal has become decomposed, which is rather early. If suddenly quenched after this first treatment the matrix metal would be unduly hard and brittle and hence I prefer to cool the castings through the critical range at such a speed as to secure toughness rather than hardness, since toughness has always been the absent feature in brakeshoes and hardness can always be secured by shortening the previous heat treatment. It is especially important that the high-temperature treatment be not too long continued, since it is important that the brakeshoes should not show the conditions characteristic of malleable iron. It is important that the brakeshoes possess a considerable proportion of combined carbon.

In the drawing accompanying and forming a part of this application Fig. 1 is a side elevation and Fig. 2 is a longitudinal section through a brakeshoe in which my improvements are or may be embodied; Fig. 3 is a cross sectional view on the line 3—3 of Fig. 1; Fig. 4 is a longitudinal sectional view of a brakeshoe containing a modified form of my invention; Fig. 5 illustrates a

third form of my invention before heat treating and Fig. 6 the same after heat treatment; Fig. 7 shows the relation of toughness to time of treatment in the case of the same composition of unstable or chilled white-iron subjected to different temperatures; and Fig. 8 shows similar data in respect of stable white-iron.

While my invention is applicable to any kind or shape of deceleration element acting frictionally, I have here chosen for illustration a common freight-car type comprising a cast-iron body 1 cast on an arcuate steel back 2 and attaching lug 3. While my improvements may enable the omission of these steel members the same can be used without detriment and will still be demanded in any event for many years, even though I consider them unnecessary. When the entire article is cast in a cold metal mold from an iron alloy containing iron, silicon and carbon of the proper relative proportions as above set forth, all the carbon will be retained in combined form; and it should be noted that primary graphite, that is graphite which has originally separated out in flake form at the outset, cannot be modified; and it will also be noted that castings wherein the absence of primary graphite is caused by the essential stability of the mixture are impracticable for the purpose in view.

However, while primary graphite cannot be modified and while stable carbides cannot be broken down within my process, the casting may contain portions either of gray-iron or of stable white-iron (or both) without detriment so long as essential parts of the casting consist of the unstable white-iron. The shoe of Fig. 2 is supposed to have been cast in an all-metal mold and to have become chilled throughout. The shoe of Fig. 4 represents the condition which exists when the same is cast in a mold having metal surfaces for the back and ends and a non-chilling surface for the face, the composition of the melt being such as to be chilled only part way through. The back and ends hence show no primary graphite and in heat treatment become toughened without changing the gray-iron in any observable way. This produces a gray-iron wearing surface 5 with an integral toughened back 6 which takes the place of the steel insert, and enables an integral lug 3a also to be cast without reinforcement although I do not consider its use as incompatible with my invention.

In Fig. 5 the shoe is cast with a gray face portion 7, a chilled white back portion 8 and an intermediate mottled portion 9. Heat treatment of this kind of shoe, as I have described, produces a tough back portion 10 as shown in Fig. 6 and leaves the gray face portion 7 and intermediate portion 9 practically unchanged. This I esteem to be due to the fact that the carbide content of the portion 9 has an opportunity due to its slower cooling to segregate out some of the silicon so that the cementite thereof is more stable than that of the chilled portion 8. The advantage of such a shoe is that the more it wears the harder it gets until the intermediate layer is passed.

The curves of Fig. 7 drawn from actual tests made on brake shoes produced by my process indicates that the toughness reaches a maximum and then falls off. With continued treatment at 1800° Fahrenheit the maximum is lower and more quickly passed, at 1650° Fahrenheit it is lower and unduly long in attainment. The maximum strength is obtained by about 4 to 5 hours at about 1700° Fahrenheit, though I do not limit myself to this temperature. The curves of Fig. 15

8 were taken from the behavior of a stable white-iron which showed little or no primary graphite even when cast in a sand mold. This is the composition used for making malleable iron which 5 when completely malleableized consists only of a ferrite matrix with graphite inclusions.

It is important, however, after the termination 10 of this heat treatment to cool the brakeshoe at a proper rate. The result of quick heat treatment 15 of the unstable carbides is to produce a substance characterized by a continuous phase of a steel-like composition having rounded or nodular inclusions of graphite therein. If cooled too quickly the matrix metal will be quenched to a condition 20 of undue hardness and brittleness; if cooled too slowly (as in the usual malleableizing process) it may be converted to ferrite by the migration of its carbon to the nodules already formed.

Other procedures than the continuous process 25 furnace can be employed; for example, the castings immediately after solidifying may be piled on cars and introduced successively into chambers of the desired temperature; or with a proper control of composition they may be introduced 30 into heat insulated pits and allowed to cool gradually therein by slow dissipation of their own heat content, until they have reached a temperature around 1100° Fahrenheit. To do this successfully requires such a composition as shall 35 cast white in the first step, and shall during this prolonged cooling period break down only part way into free carbon.

I do not limit myself to the composition above 35 specified. I have used:

|                 | A            | B            | C            |
|-----------------|--------------|--------------|--------------|
| Carbon.....     | 2.80 to 3.10 | 3.00 to 3.25 | 3.25 to 3.50 |
| Silicon.....    | .90 to 1.20  | .80 to 1.00  | .70 to .90   |
| Iron.....       | Balance..... | Balance..... | Balance..... |
| Sulphur.....    | Up to .20    | Up to .20    | Up to .20    |
| Phosphorus..... | Up to .60    | Up to .60    | Up to .60    |
| Manganese.....  | Up to 1.00   | Up to 1.00   | Up to 1.00   |

I have also used other alloying constituents 45 such as are called "hardeners" and "softeners". Such hardeners as chromium, vanadium, manganese or molybdenum render the cementite harder to break down and increase the time and temperature required. They also tend to neutralize the effect of the silicon and enable more silicon to be used (and also more carbon) without producing initial gray iron. Such softeners as nickel or aluminum may reduce the amount 50 of silicon (or carbon) permissible or reduce the time or temperature of treatment. Any cast iron 55 foundry master will understand the requirements, and in speaking of cast iron I do not exclude the use of those minor ingredients in usual proportion.

60 My improved brakeshoes, although identical with cast iron in chemical composition, exhibit a behavior equal to that of cast iron in respect of friction-coefficient and superior thereto in wear resistance, combined with a notable degree of toughness. They bend before breaking, and can 65 be dented, upset, and peened over by hammering.

As a result of this toughness and strength it becomes possible to wear these shoes almost through 70 prior to their breaking, and to dispense with all reinforcements in the form of steel backings, steel lugs, cast inserts and other inclusions, while greatly reducing the cost of replacement and the danger of failure in use, although all of these 75 known inclusions can still be employed if desired.

I do not limit myself to continuous production method or to the chill-cast method. It is possible to allow the articles to cool to seasonal temperatures and subsequently reheat them to the graphitizing temperature, and this indeed may be 80 indispensable to some plants not equipped with continuous-production mechanism.

I have referred herein to railway brakeshoes in 85 describing the invention but it is not limited to such shoes and may be used wherever a braking effect is desired, although the special advantages of the invention in an arcuate shoe and in one subjected to the severe service conditions of railway brakeshoes will be apparent.

In general I do not limit myself in any wise 90 excepting as recited in my several claims which I desire may be construed broadly each independently of limitations contained in other claims.

I claim:

1. A heat-treated brake shoe of integral section 95 and consisting of gray cast iron containing flake graphite in the wearing portion and cast iron containing nodular graphite in the other portions wherein not more than a substantially negligible proportion of graphite occurs in flake 100 form.

2. A heat-treated brake shoe of integral section 105 and made of cast iron, the body of the shoe being characterized by the occurrence of primary graphite in flake form, and the back and ends of the shoe being characterized by the occurrence of substantially all of the graphite in nodular form.

3. A heat-treated cast iron brake shoe of integral section wherein substantially all of the carbon in the wearing portion occurs in the form 110 of flake graphite and wherein a part of the carbon in the portions other than the wearing portion occurs in the form of cementite and part in the form of nodular graphite and substantially none in the form of flake graphite.

4. A heat-treated brake shoe of integral section 115 and made of cast iron containing from 2.20% to 3.50% carbon and from 1.25% to .70% silicon and wherein substantially all the graphite in the portions other than the wearing portion occurs in nodular form.

5. A brake shoe of integral section and consisting of gray cast iron containing flake graphite in the wearing portion and cast iron in the other portions wherein substantially all of the 125 graphite occurs in nodular form, the shoe having been heated to a temperature between 1600° Fahrenheit and 1800° Fahrenheit and slowly cooled through the critical range.

6. A brake shoe of integral section and consisting of gray cast iron containing flake graphite in the wearing portion and cast iron in the other portions wherein substantially all of the graphite occurs in nodular form, the shoe having been heated to a temperature between 1600° 130 Fahrenheit and 1800° Fahrenheit for a period of from fifteen minutes to eight hours and slowly cooled through the critical range.

7. A brake shoe of integral section and consisting of gray cast iron containing flake graphite in the wearing portion and cast iron containing from 2.20% to 3.50% carbon and from 1.25% to .70% silicon in the other portions wherein substantially all of the graphite occurs in nodular form, the shoe having been heated to a temperature between 1600° 145 Fahrenheit and 1800° Fahrenheit and slowly cooled through the critical range.

8. A brake shoe of integral section and consisting of gray cast iron containing flake graph-

ite in the wearing portion and cast iron containing from 2.20% to 3.50% carbon and from 1.25% to .70% silicon in the other portions wherein substantially all of the graphite occurs in nodular form, the shoe having been heated to a temperature between 1600° Fahrenheit and 1800° Fahrenheit for a period of from fifteen minutes to eight hours and slowly cooled through the critical range.

10 9. A brake shoe of integral section and consisting of cast iron containing from 2.20% to 3.50% carbon and from 1.25% to .70% silicon, the cast iron in the wearing portion of the shoe containing flake graphite, the cast iron in the ends, back and lug portion of the shoe having substantially all of the graphite occurring in nodular form, the shoe having been heated to a temperature of approximately 1700° Fahrenheit for about four or five hours and slowly cooled through the critical range.

15 10. The process of making a brake shoe which contains the steps of first casting an unstable mixture of iron, carbon and silicon under conditions which shall restrict the formation of primary graphite in the portions of the shoe other than the wearing portion, and heating the casting a period of approximately one to six hours at a temperature between 1600° and 1800° Fahrenheit to decompose the cementite in said portions at least in part with liberation of secondary graphite.

20 11. The process of making a brake shoe which contains the steps of first casting an unstable mixture of iron, carbon and silicon under conditions which shall restrict the formation of primary graphite in the portions of the shoe other than the wearing portion, heating the casting a period of approximately one to six hours at a temperature between 1600° and 1800° Fahrenheit to decompose the cementite in said portions at least in part with liberation of secondary graphite and, finally cooling at such a rate as to produce pearlitic cementite in the matrix metal.

25 12. The process of making a brake shoe which

consists in the steps of first casting the same in white iron containing from 2.20% to 3.50% carbon, from 1.25% to .70% silicon, and iron under conditions which restrict the formation of primary graphite in the portions of the shoe other than the wearing portion and which permit the formation of primary graphite in the wearing portion, subsequently heating the casting for a period of approximately four to five hours at a temperature about 1700° Fahrenheit to decompose the cementite in the portions of the shoe other than the wearing portion at least in part with the liberation of secondary graphite in the form of compact nodules of irregular outline embraced by a matrix, and finally cooling at such a rate as to produce pearlitic cementite in the matrix without materially affecting the wearing portion of the shoe.

30 13. The process of making a brake shoe which consists in the steps of first casting the same in white iron containing from 2.20% to 3.50% carbon and from 1.25% to .70% silicon and in chilling the portions of the shoe other than the wearing portion, subsequently maintaining the shoe at a temperature between 1600° Fahrenheit and 1800° Fahrenheit for a period of time to decompose the cementite in said portions at least in part with the liberation of secondary graphite in nodular form, and in finally cooling the shoe through the critical range.

35 14. The process of making a brake shoe which consists in the steps of first casting the same in white iron containing from 2.20% to 3.50% carbon and from 1.25% to .70% silicon and in chilling the portions of the shoe other than the wearing portion, subsequently maintaining the shoe at a temperature between 1600° Fahrenheit and 1800° Fahrenheit for a period of time of from fifteen minutes to eight hours to decompose the cementite in said portions at least in part with the liberation of secondary graphite in nodular form, and in finally cooling the shoe through the critical range.

FRANK A. FAHRENWALD.

45

120

50

125

55

130

60

135

65

140

70

145

75

150